

## UNITED STATES PATENT OFFICE

2,084,352

## LUBRICATING OIL

Leo Liberthson, New York, N. Y., assignor, by  
mesne assignments, to Standard Oil Develop-  
ment Company

No Drawing. Application October 2, 1934,  
Serial No. 746,515

5 Claims. (Cl. 87—9)

This invention relates to improved lubricating oils and a process of preparing same, and especially to lubricating oils having a low pour point, and being substantially non-emulsifiable.

5 Lubricating oils, and especially lubricating oils containing wax or waxy hydrocarbons in solution, tend to have a high pour point. In the case of lubricating oils containing wax or waxy hydrocarbons, the latter compounds have a tendency 10 to precipitate when the oil is cooled, thereby causing the oil to set or gel, and causing the oil to flow sluggishly or not at all. Lubricating oil distillates derived entirely or principally from the distillation of so-called Pennsylvania crude 15 oil belong generally to the waxy class mentioned.

It is known that the addition of small amounts of voltol (an oil which has been polymerized by the action of a silent electrical discharge) to a lubricating oil will lower the normal pour point 20 of such oil. However, the presence of such voltol in lubricating oils is in many cases disadvantageous in one important respect, viz; the tendency of such a mixture to permanently emulsify with water. When such a mixture is used as a lubricating oil in apparatus where it comes in contact with water, for example, in a turbine or in 25 a crank-case, the mixture forms an emulsion with the water, which raises the pour point of the lubricant and gives poor lubrication.

30 This tendency to emulsify is due to the fact that voltol is in reality a blend of mineral and vegetable oil, such blend having been found to be infinitely more susceptible to polymerization by means of a silent electrical discharge than mineral oil alone. The mineral oil can be designated 35 as the unsaponifiable component and the vegetable oil as the saponifiable component of the original voltol.

I have discovered that if the mineral oil and 40 fat constituent (the non-emulsifiable constituent) of voltol be separated from the voltol, such constituent may be added to a lubricating oil without the disadvantages attending the use of the original voltol. This may be understood from 45 the behavior of the so modified oil by subjecting it to the well known "A. S. T. M." demulsibility test. In this test steam is conducted into a definite amount of oil and permitted to condense 50 for a definite period of time. The mixture of oil and condensate should then separate into two

layers within a specified time of not more than ten minutes.

Two different types of voltol, differing only in the relative proportions of mineral oil to vegetable oil, were treated according to this invention; one a Belgian voltol sold under the trade name of "Electrion" and a second, German voltol, designated "End voltol." The physical characteristics of these two voltols are as follows:—

|                      | "Electrion"                        | "End voltol"                        | 10 |
|----------------------|------------------------------------|-------------------------------------|----|
| Gravity              | 23.1 A. P. I.                      | 18.3 A. P. I.                       |    |
| Vis. Saybolt 210° F. | 733 sec.                           | 975 sec.                            |    |
| Pour test            | 40° F.                             | 15° F.                              | 15 |
| Flash point          | 410° F.                            | 400° F.                             |    |
| Fire point           | 465° F.                            | 445° F.                             |    |
| Color                | 20 yellow 5<br>red $\frac{1}{2}$ " | 20 yellow 14<br>red $\frac{1}{2}$ " |    |
| Acidity              | 0.63 mg. KOH                       |                                     |    |
| Alkalinity           | 0.47                               |                                     |    |
| Iodine value         | 35.2                               | 17.8                                |    |
| Saponification No.   | 74.7                               | 10.0                                | 20 |
| Ash                  | 0.039%                             |                                     |    |

Each type of voltol was subjected to the action of organic solvents containing less than six carbon atoms such as normal butyl alcohol, acetone, isopropyl alcohol, isoamyl alcohol, dichloroethyl ether, etc.

For example, the voltols were treated with five volumes of butyl alcohol, preferably by counter current extraction, until 85% of the initial quantity of voltol was extracted. The residue left was a yellow, rubbery, gelatinous substance, difficultly soluble in mineral oil, but sufficiently so to act as an extremely powerful emulsifying agent.

The butyl alcohol solution of the residue-free voltol yields, after removal of the solvent an oil of the following characteristics as compared with those of the untreated voltol:

|                          | N-Butyl alcohol extract            | Original voltol                    | 40 |
|--------------------------|------------------------------------|------------------------------------|----|
| Gravity                  | 22.7 A. P. I.                      | 23.1 A. P. I.                      |    |
| Viscosity (Say.) 210° F. | 103 sec.                           | 733 sec.                           |    |
| Pour point               | 25° F.                             | 40° F.                             |    |
| Flash point              | 410° F.                            | 410° F.                            |    |
| Fire point               | 470° F.                            | 465° F.                            | 45 |
| Color                    | 20 yellow 8<br>red $\frac{1}{2}$ " | 20 yellow 5<br>red $\frac{1}{2}$ " |    |
| Acidity                  | 0.95 mg.                           | 0.63 mg.                           |    |
| Alkalinity               | 0.64 mg.                           | 0.47 mg.                           |    |
| Iodine value             | 30.2                               | 35.2                               |    |
| Saponification No.       | 63.5                               | 74.7                               | 50 |

Ordinary voltol and unemulsifiable voltol according to this invention were added to lubricating oils having the following characteristics:

5 An S. A. E. 40 blend of Pennsylvania residual and neutral oil having:

|                             |                       |
|-----------------------------|-----------------------|
| Specific gravity            | 28 A. P. I.           |
| Viscosity (Say.) at 210° F. | 79 sec.               |
| Flash point                 | 450° F.               |
| Fire point                  | 515° F.               |
| 10 Color (Lovibond)         | 20 yellow 38 red 1/2" |
| Pour point                  | 25° F.                |

When 0.5, 1, 5 and 10% of ordinary voltol were added, the pour points of the mixtures were lowered to 10, -5, -10, and -10° F. respectively, the other factors remaining substantially the same. Demulsibility tests of the mixtures however were all above 10 minutes. With the same amounts of solvent extracted unemulsifiable voltol, the same lowering of the pour points resulted, but in each of the latter cases, demulsibility occurred in less than one minute.

20 A Pennsylvania distillate having:

|                             |              |
|-----------------------------|--------------|
| 25 Specific gravity         | 29 A. P. I.  |
| Viscosity (Say.) at 210° F. | 200-205 sec. |
| Flash point                 | 420° F.      |
| Fire point                  | 470° F.      |
| Pour point                  | 30-35° F.    |

30 When 0.5, 1, 5 and 10% of ordinary voltol were added, the pour points of the mixtures were lowered to 5, -5, -10 and -10° F. respectively, the other factors remaining substantially the same. Similar pour point depressing values were obtained with similar amounts of solvent extracted unemulsifiable voltol. However, with ordinary voltol, demulsibility tests were over ten minutes, while with unemulsifiable voltol, demulsibility occurred in less than one minute.

40 A Pennsylvania distillate having:

|                             |              |
|-----------------------------|--------------|
| Specific gravity            | 30 A. P. I.  |
| Viscosity (Say.) at 210° F. | 145-150 sec. |
| Flash point                 | 405° F.      |
| Fire point                  | 460° F.      |
| Pour point                  | 10° F.       |

50 With 0.5, 1, 5 and 10% of ordinary voltol, the pour points of the mixtures were lowered to -5, -15, -25 and -25° F. respectively, the other factors remaining substantially the same. Demulsibility tests of the mixtures in each case, however, were above ten minutes. With similar amounts of solvent extracted unemulsifiable voltol, similar lowering of the pour points resulted, but in each case demulsibility occurred in less than one minute.

55 It will be noted that the Saybolt viscosity at 210° F. of the butyl alcohol extract is 103° as against 733° for the original voltol. This striking difference I believe confirms my theory that it is the higher molecular weight polymers which are responsible for the emulsifying action of voltol. It is the nature of such highly associated molecules, being relatively insoluble, to assume 60 the form of a highly dispersed and swollen colloid thus imparting a high viscosity to the external phase, in this case, the oil, and acts as a powerful emulsifying agent when water is introduced in said external phase.

65 70 The amount of solvent extract, (mineral oil and fat constituent) to be added will vary from 0.2

up to 10% of the total and will, in general, be sufficient to produce a reduction in pour test or pour point of from 10 to 50° F. Within these limits the amount added has no appreciable influence on viscosity. For a reduction in pour test of about 15° F., say from 25 to 10° F., one-half of 1% is ordinarily sufficient; and for a reduction of 25° F., say from 25° to 0° F., 1% will ordinarily be sufficient.

75 My invention includes all lubricating oils containing wax or crystallizable hydrocarbons, and I claim broadly a lubricating oil having a normal pour point and containing voltol free from its emulsion forming constituent, in an amount and potency sufficient to reduce the normal pour point 15 of the lubricating oil, the product being substantially non-emulsifiable. By non-emulsifiable I mean the product when subjected to the "A. S. T. M." demulsibility test will separate into two well defined layers in less than ten minutes. 20 I claim:

1. A product comprising a lubricating oil having a pour point caused by wax therein, and up to about 10% of a polymerized oil free from the residue insoluble in butyl alcohol, said polymerized oil being present in potency sufficient to appreciably lower the normal pour point of said lubricating oil, said polymerized oil being prepared by the action of a silent electrical discharge. 30

2. A product comprising a lubricating oil having a pour point caused by wax therein, and up to about 10% of a polymerized oil free from the residue insoluble in butyl alcohol, said polymerized oil being present in potency sufficient to lower 35 the normal pour point of said lubricating oil at least 10° F., said polymerized oil being prepared by the action of a silent electrical discharge.

3. A product comprising a lubricating oil having a pour point caused by wax therein, and up 40 to about 10% of the mineral oil and fat constituent of a polymerized oil free from the residue insoluble in butyl alcohol, said polymerized oil being present in potency sufficient to appreciably lower the normal pour point of said lubricating 45 oil, said polymerized oil being prepared by the action of a silent electrical discharge, said product being substantially non-emulsifiable.

4. A product comprising a lubricating oil having a pour point of at least 10° F. caused by wax 50 therein, and up to about 10% of the mineral oil and fat constituent of a polymerized oil free from the residue insoluble in butyl alcohol, said polymerized oil being present in potency sufficient to lower the normal pour point of said lubricating 55 oil at least 10° F., said polymerized oil being prepared by the action of a silent electrical discharge, said product being substantially non-emulsifiable.

5. A product comprising a petroleum lubricating oil distillate having a pour point of at least 10° F., caused by wax therein, and up to about 10% of the mineral oil and fat constituent of a polymerized oil free from the residue insoluble in butyl alcohol, said polymerized oil being present in 65 potency sufficient to lower the normal pour point of said distillate at least 10° F., said polymerized oil being prepared by the action of a silent electrical discharge, said product being substantially non-emulsifiable. 70

LEO LIBERTHSON.